# EUROPEAN PATENT SPECIFICATION

(11) **EP 0 255 318 B1**
(45) Date of publication and mention of the grant of the patent: **04.09.1991**
(21) Application number: 87306604.7
(22) Date of filing: 27.07.1987
(51) Int. Cl.: D21H 17/00

(54) **Method of making a water laid fibrous web containing one or more fine powders**
Verfahren zur Herstellung einer ein oder mehrere feine Pulver enthaltenden, wassergelegten Faserbahn
Procédé de fabrication d'une feuille fibreuse déposée par voie humide contenant une ou plusieurs poudres fines

(30) Priority: 31.07.1986 GB 8618733
(43) Date of publication of application: 03.02.1988
(73) Proprietor: The Wiggins Teape Group Limited, Basingstoke Hampshire RG21 2EE (GB)
(72) Inventor: Willis, Anthony John, Marlow Buckinghamshire SL7 1TX (GB); Radvan, Bronislaw, Flackwell Heath Buckinghamshire (GB)
(74) Representative: Bridge-Butler, Alan James

(56) References cited:
- EP-A- 0 148 760
- GB-A- 448 138
- US-A- 3 205 085

## Description

This invention relates to a method of making a water laid fibrous web such as a paper web or a web of plastics material and reinforcing fibres for consolidation or moulding into a fibre reinforced plastics sheet or article.

In paper webs, it is frequently necessary to incorporate particulate materials or powders such as pigments and fillers. In the case of webs of plastics material and reinforcing fibres one or more kind of particulate plastics material may be included, together with materials such as pigments, fillers and antioxidants in the form of powders of substantially smaller particle size than the plastics material.

US-A-3 205 085 is directed to a technique for enhancing the retention of titanium dioxide in paper. Prior to introduction into the papermaking stock, the titanium dioxide and sodium carboxymethylcellulose are ground together in a swing hammer mill. This process produces an intimate mixture of the two materials, with the particles being of substantially the same size.

GB-A-448 138 is concerned with a filler composition for paper, and, more particularly a composition which enhances the retention of the filler in paper. To achieve this alkaline and acid materials (lime and alum) are first reacted together in water in which a filler, which may be clay or a pigment such as titanium dioxide, is also present. This reacted mixture produces a thick pasty material which is then added to the papermaking stock before the sheet is laid down.

The process for making water laid webs requires as a prerequisite the formation of an aqueous dispersion of the fibres and particulate materials from which the web is to be formed. Preferably, a foamed dispersion is used as described in the Applicants' EP-A-0 148 760), the subject matter of that Application being incorporated by reference herein. The dispersion so formed is then drained on a foraminous support such as the Fourdrinier wire of a paper machine, to form the web.

Two problems arise in the mechanism of more than one particulate material in an aqueous or foamed dispersion as referred to above.

First, the electrochemical conditions within such dispersions make it difficult to achieve a homogeneous mixture of the various components within the dispersion, and this is reflected as a lack of homogeneity in the web as laid down on the foraminous support.

Secondly, there will be a tendency for the particulate material to be lost during the wet laying process depending on the relative dimensions of the powder particles and the apertures in the foraminous element, for example the mesh size of a Fourdrinier wire.

When certain particles or fibres are dispersed in water, it is thought that an aqueous film forms around each individual particulate or fibre and sets up an electrochemical regime such as that other particles are repelled. As a result, when fine powders are added individually, they do not agglomerate either with themselves or with other solid components of the dispersion. Thus, when the dispersion is laid down on the Fourdrinier wire, the fine particles pass through the wire with the water as drainage.

The invention is particularly concerned with a technique which will improve the homogeneity of the dispersion and resulting sheet, and which, where larger and smaller particles need to be incorporated in the sheet, will increase the retention of the smaller particles where the relative mesh size is such that they would otherwise be substantially lost in drainage through the foraminous element.

According to the present invention a method of making a web of reinforcing fibres containing in its interstices particles of at least one plastics material coated with at least one kind of powdered material substantially finer than the particulate plastics, comprises the steps of mixing the plastics particles and powdered material together in a substantially dry condition to cause the powdered material to coat the plastics particles, dispersing said coated plastics particles, together with the reinforcing fibres in water to form an aqueous dispersion, and draining the aqueous dispersion to form a web.

Thus, if a fibrous reinforced plastics material web is being made, the particulate materials can be a mixture of particulate thermoplastics. Alternatively a thermoplastic or a thermosetting polymer, can be mixed with a fine powder such as carbon black or titanium dioxide, the dry mix being dispersed in an aqueous dispersion of fibres prior to drainage to form a web. The fibres may, for example, be glass fibres.

The method of the invention is suitable for use with the process for forming a fibrous web set forth in the Applicants' EP-A-0 148 760 the subject matter of that Application being incorporated by reference herein.

Again, the invention can be employed in the manufacture of a web in which the particulate material is a fibre, the dry mix being used to form an aqueous dispersion of fibres and drained to form a web.

The method can also be employed where two or more different fibres are to be incorporated in a web, with one or more of the fibres acting as the particulate material which is dry pre-mixed with the dry fine powder before an aqueous dispersion is formed.

It has been found that when mixed dry the homogeneity of the web is improved. Also, it has been found that dry mixing causes fine powder to adhere to substantially coarser particulate material such as thermoplastic, and that this adhesion persists when the dry mix becomes part of or forms the aqueous dispersion. Since the fine powder thus becomes part of a substantially larger agglomerated component of the dispersion, it is retained in the web.

It has also been found that the invention provides a successful method of incorporating a fine pigment powder in the web so as to effect a very uniform coloration of mouldings produced using the fibrous web produced by the process, although other fine powders for other purposes such as antioxidants can of course be employed alternatively or in addition to pigments.

It will be appreciated that the method can also be employed in the manufacture of paper to enhance the retention of powdered additives.

The fine powder and particulate materials can conveniently be pre-mixed in mixers of the high shear type.

The invention can be performed in various ways and one embodiment will now be described by way of example and with reference to the accompany flow chart, which shows the benefits of the present invention by comparison with known technology.

The flow chart relates to the production of a foamed aqueous dispersion for use in the manufacture of a pigmented web of reinforcing fibre and particulate plastics material as described and claimed in EP-A-0 148 760.

The technique shown may be used for the production of dispersions of two or more particulate plastics materials so as to achieve a homogeneous mixture or of one or more particulate materials with much finer powders of, for example, pigments or antioxidants so as to achieve both homogeneity and retention of the powder during the wet web laying process.

However to illustrate the invention in a comprehensive manner the flow chart shows the technique of the invention as used for mixing two particulate polymers of relatively coarse particle size, for example, 100 to 500 µm, with a pigment having a particle size of, for example, 10 to 100 µm.

As shown in solid lines in the flow chart, the two particulate plastics materials and the pigment are first charged into a high shear powder blender 1, for example a Winkworth Ribbon Refiner Batch Mixer, a Gloucester Materials Handling High Shear Batch Blender or a Continuous Gerick E Blender (Powteck Type GAL 351). Microdiagram 2 shows that after blending the two particulate plastics materials 3a and 3b are evenly mixed and that they are both coated with the pigment 4.

The pigment coated particles 3a and 3b are transferred to a hydropulper 5 in which a foamed aqueous dispersion of glass fibres 6 has previously been formed. Because of the homogeneous mixing which has previously taken place in the mixer 1, the homogeneity of the dispersion of fibres and particles thus formed in the hydropulper 5 is assured. Furthermore, substantially all of the powdered pigment 4 continues to adhere to the larger polymeric particles 3a and 3b, as best seen in microdiagram 7.

The foamed aqueous dispersion formed in the hydropulper 5 is then used in the formation of a wet laid web in the process 8 which is carried out according to the process described in the aforementioned European Patent Application. The resulting web comprises well distributed glass fibres and polymeric particles, with the polymeric particles still retaining adherent pigments as best seen in microdiagram 9.

The formed web is then passed to drying, pressing and moulding stages 10 as required, which do not form part of this invention.

If the two particulate polymers 3a and 3b and the pigment 4 are added directly to the hydropulper 5 as indicated by the broken lines 11 and not premixed in a substantially dry state in the mixer 1, it is more difficult to achieve homogeneous mixing with the fibres 6 in the dispersion. Furthermore, the powdered pigment becomes dispersed as individual particles in the foamed dispersion, as best seen in microdiagram 12. As a result they tend to be lost in drainage during the wet laying process, so that few or none remain in the formed web, as shown in microdiagram 14.

It will be appreciated that the materials which can be premixed as described are not limited to particulate polymers or pigments. Wood or glass fibres, clays and other fillers are understood as falling within the scope of the term "particulate materials" which can be so premixed.

Where plastics materials are to be included, they may comprise thermoplastics or thermosetting plastics particles of various kinds alone or as blends with other plastics for example as follows:
Acrylonitrile-butadiene-styrene with Polyvincylchloride
Acrylonitrile-butadiene-styrene with Polypropylene
Polyphenylene ether with Polypropylene
Polyphenylene ether with Polyamide
Polycarbonate with Polyalkyleneterephthalate
Polycarbonate with Polyestercarbonate
Polyvinylchloride with Phenolformaldehyde
Polypropylene with Lignin

Where such polymers are incorporated alone or as blends, finely powdered antioxidants may be adhered to them by premixing as above described, together with, if desired, pigments such as carbon black or titanium dioxide or fillers such as calcium carbonate. Alternatively, or in addition, one of two particulate polymeric plastics to be included may be first ground to a smaller dimension and then adhered to the other plastic by premixing as above described.

As referred to earlier the particulate material can be the fibres themselves and thus the invention can be used in a paper making process by mixing the fine powder, again, for example a colouring pigment, with the fibres, for example, cellulose fibres in dry form and then using the mix to form an aqueous dispersion, laying this on a wire and forming a paper web in the usual manner.

The process can also be used if more than one kind of fibre is employed in a web, the fine powders being dry mixed with one or more of the fibres to be used prior to forming the aqueous dispersion.

## Claims

1. A method of making a web of reinforcing fibres containing in its interstices particles of at least one plastics material coated with at least one kind of powdered material substantially finer than the particulate plastics, comprising the steps of:
mixing the plastics particles and powdered material together in a substantially dry condition to cause the powdered material to coat the plastics particles,
dispersing said coated plastics particles, together with the reinforcing fibres in water to form an aqueous dispersion, and
draining the aqueous dispersion to form a web.

2. A method as claimed in claim 1, in which the aqueous dispersion is foamed.

3. A method as claimed in claim 1 or claim 2, in which the particulate plastics material comprises a thermoplastic or thermosetting polymer.

4. A method as claimed in any one of the preceding claims in which at least one of the powdered materials is a pigment.

5. A method as claimed in claim 4 in which the pigment is carbon black or titanium dioxide.

6. A method as claimed in any one of the preceding claims 1 to 3 in which at least one of the powdered materials is an anti-oxidant for one of the plastics materials.

7. A method as claimed in any one of the preceding claims in which the fibres are glass fibres.

8. A fibrous web comprising a matrix of reinforcing fibres having in the interstices thereof particles of at least one plastics material, said particles each being coated with at least one powdered material substantially finer than said particles.

## Revendications

1. Procédé de fabrication d'une feuille de fibres de renforcement contenant dans ses interstices des particules d'au moins une matière plastique revêtues d'au moins un type de matière en poudre essentiellement plus fine que les matières plastiques particulaires, consistant à :
mélanger des particules de matière plastique et de matière en poudre à l'état essentiellement sec pour revêtir les particules de matière plastique,
disperser lesdites particules de matière plastique revêtues, avec les fibres de renforcement, dans l'eau pour former une dispersion aqueuse, et
égoutter la dispersion aqueuse pour former une feuille.

2. Procédé selon la revendication 1, dans lequel la dispersion aqueuse est sous forme de mousse.

3. Procédé selon la revendication 1 ou la revendication 2, dans lequel la matière plastique en particules comprend un polymère thermoplastique ou thermodurcissable.

4. Procédé selon l'une quelconque des revendications précédentes dans lequel au moins une des matières en poudre est un pigment.

5. Procédé selon la revendication 4 dans lequel le pigment est le noir de fumée ou le dioxyde de titane.

6. Procédé selon l'une quelconque des revendications 1 à 3 précédentes dans lequel au moins une des matières en poudre est un anti-oxydant pour une des matières plastiques.

7. Procédé selon l'une quelconque des revendications précédentes dans lequel les fibres sont des fibres de verre.

8. Feuille fibreuse comprenant une matrice de fibres de renforcement ayant dans ses interstices des particules d'au moins une matière plastique, lesdites particules étant chacune revêtues d'au moins une matière en poudre essentiellement plus fine que lesdites particules.

## Patentansprüche

1. Verfahren zur Herstellung einer Bahn mit verstärkenden Fasern, welche in ihren Zwischenräumen Partikel von mindestens einem Kunststoffmaterial enthalten, das mit mindestens einer Art von Pulverisiertem Material beschichtet ist, das im wesentlichen feiner ist als der aus Partikeln bestehende Kunststoff, das folgende Schritte umfaßt: zusammenmischen der Kunststoffpartikel und des pulverisierten Materials in einem im wesentlichen trockenen Zustand, um zu veranlassen, daß das pulverisierte Material die Kunststoffpartikel überzieht,
dispergieren der beschichteten Kunststoffpartikel zusammen mit den verstärkenden Fasern in Wasser zur Bildung einer wässrigen Dispersion und
entwässern der wässrigen Dispersion zur Bildung einer Bahn

2. Verfahren nach Anspruch 1, bei welchem die wässrige Dispersion geschäumt ist

3. Verfahren nach Anspruch 1 oder 2, bei welchem das aus Partikeln bestehende Kunststoffmaterial ein thermoplastisches oder ein duroplastisches Polymer umfasst.

4. Verfahren nach einem der vorhergehenden Ansprüche, bei welchem das mindestens eine pulverisierte Material ein Pigment ist

5. Verfahren nach Anspruch 4, bei welchem das Pigment mit Carbon Black oder Titandioxid ist

6. Verfahren nach einem der vorstehenden Ansprüche 1 bis 3, bei welchem das mindestens eine pulverisierte Material ein Antioxydanz für eines der Kunststoffmaterialien ist

7. Verfahren nach einem der vorhergehenden Ansprüche, bei welchem die Fasern Glasfasern sind

8. Fasrige Bahn, welche eine Matrix von verstärkenden Fasern aufweist, welche in ihren Zwischenräumen Partikel von mindestens einem Kunststoffmaterial aufweisen, wobei jedes der Partikel mit mindestens einem pulverisierten Material beschichtet ist, das im wesentlichen feiner ist als die Partikel
